

Patented Nov. 29, 1949

2,489,249

# UNITED STATES PATENT OFFICE

2,489,249

## LUBRICANT

David E. Adelson, Berkeley, Calif., assignor to  
Shell Development Company, San Francisco,  
Calif., a corporation of Delaware

No Drawing. Application March 31, 1947,  
Serial No. 738,495

20 Claims. (Cl. 252—46.6)

1

This invention relates to novel reaction products having properties of greatly improving and stabilizing lubricants, and is a continuation-in-part of my pending application, Serial No. 718,617, filed December 26, 1946. This invention also pertains to lubricants, such as mineral lubricating oils, synthetic lubricants of hydrocarbon or non-hydrocarbon origin, and the like, containing therein a multi-functional additive having detergent and anti-ringsticking properties, as well as acting as an inhibitor of oxidation and corrosion.

It is well known that various lubricants whether doped or undoped, tend to oxidize and to form corrosive bodies and sludge, when used in modern engines and machines operating under ordinary conditions or at high speeds, elevated temperatures, heavy loads and/or other adverse conditions. Some of the deterioration products of lubricants formed during their use are hard carbonaceous materials which adhere to metal surfaces and causes scratching and scuffing of movable metal parts and the sticking of valves and piston rings in engines. In addition, presently known lubricants are generally incapable of maintaining a continuous lubricating film between movable metal parts, resulting in gradual or rapid wearing away of metal parts. The damage thus caused required replacement of such parts or even the complete overhauling of engines and machines, resulting in expensive loss of production and time.

In the case of the highest quality non-corrosive, stable lubricating oils, which have been highly refined for specific uses, or synthetic lubricants developed for specific or special uses, it has been observed that such oils or lubricants are generally highly susceptible to oxidation and deterioration, becoming progressively more corrosive in engines and machines even under ordinary operating conditions.

To improve the lubricating properties of oils and synthetic lubricants it has become the practice to blend with various lubricants, one and in most cases more than one addition agents, which additives have the effect or property of inhibiting deterioration of lubricants and impart to them certain beneficial properties. Thus, additives have been specifically designed which have the property of inhibiting corrosion of alloyed bearings such as copper-lead, cadmium-silver and the like, developed for automotive, Diesel and aircraft engines. Acidic oxidation or decomposition components formed in lubricants during use readily attack these bearings but are inhibited or prevented from doing this by the formation of a corrosion protective film formed on the bearing sur-

face with the aid of the additive. Additives have also been developed which possess the property of modifying the carbonaceous materials formed, by deterioration of lubricants, on piston rods, rings and valves, and other metal parts in internal combustion engines, automotive and truck engines, aviation engines, high speed Diesel engines and the like. Such additives serve a very important function because, by modifying this carbonaceous material so that it can be removed easily, the tendency of engine parts to become stuck is inhibited so that ringsticking, piston scuffing, scratching and wearing away of other engine parts and material reduction of engine efficiency, are prevented or materially inhibited.

Other additives have been developed for the purpose of acting as detergents in lubricants in order to assist in the removal of soot or sludge, varnish, lacquer formed from deterioration of the oil when subjected to high operating temperatures. Detergents due to their cleaning action prevent the build up of these deleterious materials and assist in removing those formed. Anti-wear additives have the property of reducing friction of movable metal parts of the same or different metals. Due to the function exerted or property imparted by such additives on lubricants, wear caused by direct frictional contact of metals can be greatly reduced. Also additives have been developed to withstand extreme pressures, disperse impurities, solubilize certain additives and the like.

The development of numerous additives has been due to the fact that most, if not all additives are capable of functioning in substantially only one specific manner. Very few lubricant additives have the ability of improving a lubricant in more than just one respect. Thus, a good antioxidant might not be able to inhibit lacquer and varnish formation on piston rods or act as a detergent or corrosion inhibitor. In many cases it is found that an additive possesses very good properties in one respect, but is the cause of harmful formations and therefore detrimental as an additive in another respect. Therefore, other additives are frequently required to obtain a good stable lubricant. The combination of additives in lubricants wherein each additive exerts its influence without interfering with the function of other additives is a difficult matter to attain. In most cases additives co-react or interfere with each other. To prevent this great care must be taken in selecting the additives, mixing them in specific proportions and continuously watching and replacing additives which have stopped functioning or have deteriorated.

It is an object of this invention to improve the lubricating properties of various lubricating bases by the addition thereto of a minor amount of a multi-functional material. Another object of this invention is to add to compounded or doped lubricants a multi-functional material whereby a synergistic effect is produced, resulting in a product of accentuated and improved properties. Another object of this invention is to add to oleaginous materials, mineral lubricating oils, synthetic lubricants and the like, a multi-functional material so as to inhibit oxidation and corrosion and prevent the formation of sludge, varnish and lacquer in said lubricants even under adverse operating conditions. Still another object of this invention is to use in lubricating compositions a multi-functional material which prevents ringsticking as well as the sticking of other engine parts due to deterioration of the lubricant. Also it is an object of this invention to use in oleaginous materials, e. g. in lubricating compositions, a multi-functional material which inhibits wear, scuffing, scratching and other damage to engine parts. Furthermore it is an object of this invention to provide novel multi-functional improving and enhancing additives for lubricating bases. Other objects of this invention will appear as the description proceeds.

To the accomplishment of the foregoing and related ends, this invention consists of features which will be hereinafter fully described, and particularly pointed out in the claims, the following description setting forth in detail certain embodiments of the invention, these being illustrative of but a few variations in which the principle of the invention may be employed.

Broadly stated, this invention is directed to the use, in lubricants, of reaction products obtained by reacting organic compounds with hydrogen sulfide in the presence of ammonium hydrosulfide and treating said reaction products with phosphorus and sulfur and/or a sulfur-containing agent, such as elemental sulfur, sulfur halides, sodium polysulfides, phosphorus sulfides, and the like. Among the organic compounds which can be used to form reaction products of this invention are:

## I. ALIPHATIC HYDROCARBONS

### *Acyclic compounds*

A. Saturated paraffinic hydrocarbons above 6 carbon atoms such as

hexane  
heptane  
octane  
nonane  
tetradecane  
hexadecane  
eicosane  
tetraicosane  
and the like.

B. Unsaturated paraffinic hydrocarbons above 6 carbon atoms such as

hexylene  
heptylene  
polyolefines  
which may be broadly termed polyalkenes, and include polypropene, polypentenes as well as branched chain unsaturated hydrocarbons such as iso-olefines and iso-polyolefines.

### *Cyclic compounds*

A. Saturated:

cyclobutane  
cyclohexane  
cyclo-octane  
and the like.

B. Unsaturated:

cyclopentadiene  
cyclohexene  
cyclo-octene  
and the like.

## II. AROMATIC HYDROCARBONS

A  
benzene  
naphthalene  
anthracene  
phenanthrene  
bi-phenyl  
di-phenylmethane  
stilbene  
and the like.

B  
alkyl  
hydroxy  
amine  
nitro  
nitroso  
halogen  
carboxyl  
mercaptan

Substituted aromatic compounds of group II A and the like.

## III. CYCLIC TERPENES

## IV. HETERO CYCLIC COMPOUNDS

|   |                                                                                                                               |    |                                                                                                                                                                      |
|---|-------------------------------------------------------------------------------------------------------------------------------|----|----------------------------------------------------------------------------------------------------------------------------------------------------------------------|
| 5 | cymene<br>limonene<br>pinene<br>bornylene<br>methene<br>terpinolene<br>terpin<br>menthol<br>menthone<br>isoborneol<br>camphor | 10 | furan, furfural,<br>furfuryl alcohol,<br>furoic acid,<br>pyrone, pyridine,<br>picolinic acid,<br>nicotinic acid,<br>pyran, morpholine,<br>coumarone<br>and the like. |
|---|-------------------------------------------------------------------------------------------------------------------------------|----|----------------------------------------------------------------------------------------------------------------------------------------------------------------------|

Both the cyclic terpenes and the heterocyclic compounds can have attached thereto substituent radicals, such as alkyl and alkenyl radicals, hydroxy and halogen groups, and the like.

## V. ALCOHOLS

|                                                       |                          |
|-------------------------------------------------------|--------------------------|
| A. Aliphatic (saturated and unsaturated):             | B. Aromatic alcohols:    |
| 20 amyl alcohol                                       | phenyl ethyl alcohol     |
| hexyl alcohol                                         | phenyl octyl alcohol     |
| heptyl alcohol                                        | octadecyl benzyl alcohol |
| octyl alcohol                                         | benzyl alcohol           |
| decyl alcohol                                         | and the like.            |
| dodecyl alcohol                                       | C. Cyclic alcohols:      |
| octadecyl alcohol                                     | naphthenic alcohol       |
| carnaubyl alcohol                                     |                          |
| oleyl alcohol                                         |                          |
| Polyhydric aliphatic alcohols:                        |                          |
| glycols                                               | mannitol                 |
| pinocols                                              | sorbitol                 |
| erythrol                                              | and the like.            |
| D. Natural occurring alcohols and synthetic alcohols: |                          |
| Alcohols as found in wool fat, sperm oil              |                          |
| Alcohols produced by oxidation of hydrocarbons, e. g. |                          |
| paraffin wax                                          |                          |
| sweat wax                                             |                          |
| petrolatum                                            |                          |
| and the like.                                         |                          |

## VI. PHENOLIC COMPOUNDS

Phenol, alkyl phenol, catechol, resorcinol, pyrogallol.

All of these compounds may contain substituent groups such as alkyl radicals, amino, halogen, carboxyl and the like, hydroquinone, quinone, ocreinol, phloroglucinol, cresols, thymol, saligenin, cinnamyl alcohol, methyl phenyl carbinol, eugenol, cardanol, etc.

### A. Aliphatic (mono and poly-carboxylic and hydroxy substituted acids and the like):

capric  
undecylic

lauric

myristic

palmitic

stearyl

arachidic acids;

acrylic

sorbic, oleic, linoleic

linolinic acids;

hydroxy stearic

di and tri hydroxy stearic

ricinoleic acids;

alkyl malonic acid

alkyl succinic acid

alkyl glutaric acid

glycolic acid

pyruvic acid

phthalonic acid

lactic acid

alkyl maleic acid

alkyl malic acid

alkyl tartaric acid

alkyl citric acid

keto acids

suberic acid

alkyl adipic acid

tartaric acid

and the like, acids produced by

oxidation of hydrocarbon, e. g.

paraffin wax and the like.

### B. Aromatic acids:

Benzoic

salicylic

cinnamic

hydrocinnamic

phthalic

naphthoic

abietic

naphthenic and sulfonic acids

derived from petroleum hydrocarbons, mandelic acid, and the like;

phenyl acetic acid

phenyl stearic acid

naphthyl stearic acid

resinic acid

## VIII. ESTERS

Esters contemplated for use in this invention may be obtained by reaction of any of the compounds listed under group V and VI and their derivatives, with any of the acids listed under group VII.

## IX. ETHERS

The ethers contemplated for use in this invention may be symmetrical, unsymmetrical, or mixed ethers of dialkyl ethers, alkyl-aryl ethers, aryl ethers and the like. Specifically it is desirable to use:

- A. Aliphatic (saturated and unsaturated):  
methyl, ethyl methyl, ethyl, ethyl propyl, isopropyl, octyl, ethers and the like; vinyl, allyl, crotonyl ethers and the like and mixture of saturated and unsaturated ethers.
- B. Cyclic and poly ethers:  
ethylene oxide, propylene oxide, acetal, dioxan and the like.
- C. Aromatic ethers:  
anisole, phenetole, diphenyl, dixenyl, dimethyl ethers, benzyl phenyl ether, benzyl ether cardoxyethanol and the like.
- D. Substituted ethers:  
alkyloxy ethers of polyhydroxy aromatics such as resorcinol, pyrogallol and the like.

## X. ALDEHYDES

- A. Aliphatic (saturated and unsaturated):  
acetaldehyde, propionaldehyde, butyraldehyde, caproaldehyde and the like; acrolein, crotonaldehyde, citral, etc.
- B. Aromatic:  
Benzaldehyde, cinnamaldehyde, salicylaldehyde, naphthaldehyde, vanillin, etc.

## XI. KETONES

- A. Aliphatic (saturated and unsaturated):  
acetone, butanone, hexanone, oleone, palmitone, methyl ethyl ketone, methyl propyl ketone, butyrone, butenone, pentanone, phorone, pentanedione, mesityl oxide, diethyl ketone, 3-methylheptanone, di-isobutyl ketone, diacetone alcohol, and the like.
- B. Aromatic:  
acetophenone, propiophenone, dibenzyl ketone, benzyl phenyl ketone, benzophenone and the like.
- C. Cyclic ketones:  
cyclobutanone, cyclopentanone, quinones, cycloheptanone  
pure isophorone and isophorone bottoms the manufacture of which will be fully described hereinafter.

## XII. NATURAL FATS, OILS AND WAXES AND THEIR DERIVATIVES AND MISCELLANEOUS COMPOUNDS

- A. Vegetable and animal oils, fats, and waxes such as:  
castor oil, coconut oil, corn oil, cottonseed oil, horse fat, lard oil, mutton tallow, beef tallow, neat's-foot oil, palm oil, peanut oil, rapeseed oil, soya bean oil, sperm oil, whale oil, wool fat, Japan wax, olefin waxes, paraffin waxes, wax tailings, petrolatum, vegetable and animal phosphatidic materials, montan wax, cannauba wax, beeswax, spermaceti, castor oil distillate, ozokerite, tall oil, and the like.

- B. Petroleum hydrocarbons such as:  
naphtha, mineral seal oil, kerosene, gas oils, etc.

XIII. Metal salts and organic bases of organic acidic materials listed in any of the above groups, their mixtures, or various combinations may be treated with hydrogen sulfide in presence of ammonium hydrosulfide. Metal bases include those of the alkali metals, Cu, Mg, Ca, Cr, Br, Zn, Cd, Al, Sn, Pb, Cr, Mn, Fe, Ni, Co, etc. Organic bases include various nitrogen bases as primary, secondary, tertiary and quaternary amines.

Among the specific and preferred compounds contemplated for reacting with hydrogen sulfide in the presence of ammonium hydrosulfide and further treating said product with either a phosphorus sulfide and/or a sulfurizing agent, may be mentioned: stilbene, oleic acid, ammonium oleate, potassium oleate, ammonium undecylenate,

ethyl undecylenate, methyl ricinoleate, cottonseed oil, rapeseed oil, peanut oil, dehydrated castor oil, and tall oil as well as wax olefins, cinnamyl alcohol, pentanedione - 2,4-diphenyl methane, high molecular weight saturated and unsaturated ketones diacetone alcohol, mesityl oxide, ethyl oleate, ethyl cinnamate, cinnamaldehyde, and isophorone bottoms, the production and identification of which latter will be fully described below.

Isophorone bottoms are primarily high molecular weight unsaturated ketones having at least 12 and preferably more than 18 carbon atoms in the molecule. These products may be obtained by condensation of acetone in a caustic solution under elevated temperature and pressure. Specifically the product is obtainable by condensing acetone in a 30% to 60% caustic solution at a temperature ranging between about 130° C. and about 170° C., and under a pressure of from about 300 to about 500 pounds per square inch. The resultant product is subjected to distillation to remove distillable ketones and other constituents and impurities. The product remaining in the still is preferably purified by filtration, solvent treatment, and comprises crude unsaturated cyclic ketones of high molecular weight, preferably referred to as "crude isophorone bottoms." The term "isophorone bottoms" as referred to herein is usually a complex mixture of high molecular weight unsaturated cyclic ketones containing at least 12 and preferably more than 18 carbon atoms in the molecule. The product thus formed is not to be confused with straight isophorone which is specifically 3,5,5-trimethyl cyclohexene-2-one-1, which is an unsaturated cyclic ketone containing only nine carbon atoms in the molecule. Isophorone bottoms produced by condensation of acetone under conditions referred to above includes within its scope any and all unsaturated cyclic ketones containing at least 12 and preferably more than 18 carbon atoms and having generally the chemical structural configuration of isophorone as well as the chemical structural configuration resulting from its further condensation.

Crude isophorone bottoms can be fractionated and/or chemically treated and each fraction therefrom can in turn be treated with ammonium hydrosulfide-hydrogen sulfide and thereafter with phosphorus sulfide and/or sulfur compounds at elevated temperatures to produce a compound containing both phosphorus and/or sulfur. Among the various fractions which can be obtained from crude isophorone bottoms are topped, crude isophorone bottoms which contain at least 18 carbon atoms in the molecular and are obtained after removal of distillate from crude isophorone bottoms to a still head temperature of 140° C. at 10 mm. mercury pressure. Another fraction of crude isophorone bottoms can be subjected to hydrolysis with dilute sodium hydroxide and the acetone and isophorone formed removed by distillation. The bottoms can then be filtered and purified and comprise essentially unsaturated cyclic ketones containing at least 12 and more carbon atoms in the molecule and are referred to as crude, hydrolyzed isophorone bottoms. This material can be subjected to distillation to split it into two fractions. The distilled hydrolyzed isophorone fraction has a boiling point of about 140° C. at 10 mm. mercury pressure and consists of a mixture of unsaturated cyclic ketones containing between 15 to 18 carbon atoms in the molecule. The residue is referred to as topped,

crude hydrolyzed isophorone bottoms and is similar to topped crude isophorone bottoms. This residue comprises essentially unsaturated cyclic ketones of at least 15 carbon atoms and higher in the molecule. Crude isophorone bottoms can be also subjected to condensation over solid sodium hydroxide to yield two types of resinous materials. The first resinous fraction or soft resin has a viscosity at 210° F. of about 25-26 centistokes and an average molecular weight of from 320 to 350. The heavier fraction or medium resin has a viscosity at 210° F. of about 80 to 120 centistokes and an average molecular weight of from 370 to 390. The unsaturated cyclic ketones can be hydrogenated to produce saturated cyclic ketones. All of the various saturated and unsaturated cyclic ketone fractions obtained in the manner described above can, in accordance with one phase of this invention, be first reacted with hydrogen sulfide in the presence of ammonium hydrosulfide, and the reaction product thus formed may then be further treated with a phosphorus sulfide and/or a sulfurizing agent to form desired final reaction products having outstanding properties as improving agents for lubricants. Among the phosphorus sulfide and/or sulfurizing agents which can be used to treat the initial reaction, namely the reaction of hydrogen sulfide-ammonium hydrosulfide and an organic compound are:  $P_2S_5$ ,  $P_4S_3$ , and/or elemental sulfur,  $SCl_2$ ,  $S_2Cl_2$ , sodium sulfide, sodium tetra-sulfide, sodium pentasulfide, and the like.

The products formed by the reaction of ammonium hydrosulfide-hydrogen sulfide with organic compound can be prepared at room or elevated temperatures, preferably in closed vessels. The use of elevated temperatures apparently only speeds up the reaction. However, the cost of fuel and special equipment outweighs this feature, and it has been ordinarily found more advantageous to simply allow the ammonium hydrosulfide-hydrogen sulfide organic compound reactions to take place at room temperature in closed vessels for the necessary period of time, e. g. from one week to one month or more, depending upon the organic material being treated. The final reaction product which is formed by treating the reaction products of ammonium hydrosulfide-hydrogen sulfide and an organic compound with any of the previously mentioned phosphorus sulfide and/or sulfurizing agents can be carried out at elevated temperatures of between about 100° C. and about 200° C. and preferably between about 150° C. and about 170° C., and if desired in the presence of a suitable inert solvent.

To more clearly illustrate the present invention, the following examples are presented. It is to be understood however that various modifications can be resorted to without departing from the spirit of the invention.

#### EXAMPLE I

##### A. Initial reaction product of hydrogen sulfide in the presence of ammonium hydrosulfide with topped, crude isophorone bottoms

Isopropyl alcohol (700 cc.) contained in a 4-liter, thick-walled suction flask, was saturated with dry ammonia followed by dry hydrogen sulfide. A solution of 238.5 grams of topped, crude isophorone bottoms in 350 cc. isopropyl alcohol was added and the resulting solution was saturated with hydrogen sulfide. The side-neck and mouth of the flask were then closed and the flask

was allowed to stand for a week with infrequent shaking. Upon opening the flask a partial vacuum was discovered. The reaction mixture was filtered to remove impurities and the isopropyl alcohol was removed from the filtrate by evaporation. The residue was dissolved in 500 cc. of a non-aromatic hydrocarbon having a boiling range of between about 164° F. and 233° F. and washed with water. After removal of the solvent in a current of nitrogen gas on a steam bath, a very viscous sticky mass was obtained, said mass possessing a pleasant odor and exhibiting much less flow at room temperature than did the starting materials. The product was oil-soluble and on analysis contained:

|                                                            | Analysis of Product | Analysis of cyclic ketone (topped, crude isophorone bottoms) |
|------------------------------------------------------------|---------------------|--------------------------------------------------------------|
| Percent by weight Sulfur.....                              | 7.2 (5)             | 79.5 (9)                                                     |
| Percent by weight Carbon.....                              | 76.2 (1)            | 79.5 (9)                                                     |
| Percent by weight Hydrogen.....                            | 9.6 (2)             | 9.8 (9)                                                      |
| Percent by weight Nitrogen.....                            | 0.26                |                                                              |
| Percent by weight Oxygen (by difference).....              | 6.6 (6)             | 10.5 (2)                                                     |
| Mol. weight (ebulliscopic determination in $C_6H_6$ )..... | 352                 | 316                                                          |

##### 30 B. Final reaction product obtained by treating (A) with phosphorus pentasulfide

To approximately one hundred grams of the above initial reaction product about 50 grams of phosphorus sulfide were slowly added and the mixture was constantly stirred and heated for about 5 hours. The heating was done by initially maintaining the temperature at about 60° C. to 80° C. and then rapidly heating to approximately 160° C. and maintaining the reaction at this temperature until completed. At the end of the reaction period, the desired product was extracted with a non-aromatic hydrocarbon having a boiling range of between about 164° F. and 233° F. The solution was filtered and the filtrate evaporated at steam temperature in a current of carbon dioxide. The resultant product was a soft, brown solid which contained 14.2% sulfur and 4.6% phosphorus.

35 The process was repeated with initial reaction products as above but having sulfur contents of (a) 3.27 to 3.28% sulfur and (b) 4.20% to 4.30% sulfur and these final phosphorus sulfide-reaction products on analysis contained:

|                                                                         |                         |
|-------------------------------------------------------------------------|-------------------------|
| Percent S in initial product (A).....                                   | 3.27 to 3.28% S by wt.  |
| Percent S and P after treating initial product<br>A with $P_2S_5$ ..... |                         |
| Percent S in final reaction product.....                                | {14.2 to 14.5% S by wt. |
| Percent P in final reaction product.....                                | {4.17 to 4.2% P by wt.  |
| Percent S in initial product (A).....                                   | 4.2 to 4.3% S by wt.    |
| Percent S and P after treating initial product<br>with $P_2S_5$ .....   |                         |
| Percent S in final reaction product.....                                | {14.3 to 15.4% S by wt. |
| Percent P in final reaction product.....                                | {4.21 to 4.6% P by wt.  |

#### EXAMPLE II

##### A. Initial reaction product of ammonium hydrosulfide-hydrogen sulfide and topped, crude isophorone bottoms

70 This reaction product was prepared in an isopropyl alcohol medium (1315 cc.) using about 295 gm. of topped, crude isophorone bottoms in an autoclave for 5½ hours at 96° C. to 101.5° C. The product was then treated as indicated in

Example I part A and the analysis of the product was as follows:

Per cent by wt. Sulfur ----- 6.2  
 Per cent by wt. Carbon ----- 77.2 (3)  
 Per cent by wt. Hydrogen ----- 9.6 (2)  
 Per cent by wt. Nitrogen ----- 0.3 (9)  
 Per cent by wt. Oxygen ----- 6.5 (6)  
 Mol. wt. ----- 356

B. Final reaction product obtained by treating 10 product as obtained under A with sulfur

To approximately 80 gms. of the above initial reaction product about 16 gm. of elemental sulfur were added and the mixture was constantly stirred and heated for 2 hours at a temperature between about 150 to 170° C. The resultant product was a dark brown very viscous mass which contained about 16.8% sulfur by weight.

The process of sulfurizing the above initial reaction product was repeated as indicated under B, except that the reaction time was increased to 4 hours and on analysis this reaction product contained 17.1% sulfur by weight.

Other phosphorus and sulfur and/or sulfur treated ammonium hydrosulfide-hydrogen sulfide-organic compound reaction products which are particularly preferable as lubricating oil additives are as follows:

- (1) Ammonium hydrosulfide-hydrogen sulfide-mesityl oxide treated with phosphorus pentasulfide and/or elemental sulfur.
- (2) Ammonium hydrosulfide-hydrogen sulfide-diacetone alcohol treated with phosphorus pentasulfide and/or elemental sulfur.
- (3) Ammonium hydrosulfide-hydrogen sulfide-wax olefins treated with phosphorus pentasulfide and/or elemental sulfur and/or sodium tetrasulfide.
- (4) Ammonium hydrosulfide-hydrogen sulfide-stilbene treated with phosphorus pentasulfide and/or elemental sulfur.
- (5) Ammonium hydrosulfide-hydrogen sulfide-pentandione-2,4 treated with phosphorus pentasulfide and/or elemental sulfur and/or sodium tetrasulfide and/or sulfur chloride.
- (6) Ammonium hydrosulfide-hydrogen sulfide-diphenyl methane treated with phosphorus pentasulfide and/or elemental sulfur.
- (7) Ammonium hydrosulfide-hydrogen sulfide-oleic acid treated with phosphorus pentasulfide and/or elemental sulfur and/or sodium tetrasulfide.
- (8) Ammonium hydrosulfide-hydrogen sulfide-ammonium oleate treated with phosphorus pentasulfide and/or elemental sulfur.
- (9) Ammonium hydrosulfide-hydrogen sulfide-potassium oleate treated with phosphorus pentasulfide and/or elemental sulfur.
- (10) Ammonium hydrosulfide-hydrogen sulfide-ammonium undecylenate treated with phosphorus pentasulfide and/or elemental sulfur.
- (11) Ammonium hydrosulfide-hydrogen sulfide-ethyl undecylenate treated with phosphorus pentasulfide and/or elemental sulfur.
- (12) Ammonium hydrosulfide-hydrogen sulfide-ethyl cinnamate treated with phosphorus pentasulfide and/or elemental sulfur.

- (13) Ammonium hydrosulfide-hydrogen sulfide-methyl ricinoleate treated with phosphorus pentasulfide and/or elemental sulfur.
- 5 (14) Ammonium hydrosulfide-hydrogen sulfide-cottonseed oil treated with phosphorus pentasulfide and/or elemental sulfur.
- (15) Ammonium hydrosulfide-hydrogen sulfide-rapeseed oil treated with phosphorus pentasulfide and/or elemental sulfur.
- (16) Ammonium hydrosulfide-hydrogen sulfide-peanut oil treated with phosphorus pentasulfide and/or elemental sulfur.
- (17) Ammonium hydrosulfide-hydrogen sulfide-dehydrated castor oil treated with phosphorus pentasulfide and/or elemental sulfur.
- (18) Ammonium hydrosulfide-hydrogen sulfide-tall oil treated with phosphorus pentasulfide and/or elemental sulfur.
- (19) Ammonium hydrosulfide-hydrogen sulfide-cinnamyl alcohol treated with phosphorus pentasulfide and/or elemental sulfur.
- (20) Ammonium hydrosulfide-hydrogen sulfide-cinnamaldehyde treated with phosphorus pentasulfide and/or elemental sulfur.

To illustrate the pronounced improvement obtained in lubricating compositions by the addition of small amounts of reaction products of this invention, the following test data is given:

TABLE I

## Oxidation stability determination

[A refined undoped lubricating oil, 64-67 S. U. at 210° F. was employed, temperature 150° C.]

| Additives                                                                                                                                 | Catalyst: 1 cm. <sup>3</sup> Cu/gm. oil <sup>1</sup> |                               |
|-------------------------------------------------------------------------------------------------------------------------------------------|------------------------------------------------------|-------------------------------|
|                                                                                                                                           | Amount per cent sulfate ash                          | 1500 ml. oxygen, time (hours) |
| 1 None                                                                                                                                    |                                                      | 5.9                           |
| 2 Reaction Product of Example I part A, namely, ammonium hydrosulfide-hydrogen sulfide with topped, crude isophorone bottoms              | 0.1                                                  | 13.1                          |
| 3 P <sub>2</sub> S <sub>5</sub> treated reaction product of ammonium hydrosulfide-hydrogen sulfide with topped, crude isophorone bottoms  | 0.1                                                  | 96.0                          |
| 4 Elemental sulfur treated reaction product of ammonium hydrosulfide-hydrogen sulfide with topped, crude isophorone bottoms               | 0.1                                                  | 65.6                          |
| 5 Ca salt of alkyl phenolformaldehyde condensation product                                                                                | 0.2                                                  | 14.2                          |
| 6 + Ca petroleum sulfonate                                                                                                                | 0.1                                                  |                               |
| 7 Reaction Product of Example I part A, namely, ammonium hydrosulfide-hydrogen sulfide with topped, crude isophorone bottoms              | 0.1                                                  | 13.1                          |
| 8 + Ca salt of alkyl phenolformaldehyde condensation product                                                                              | 0.2                                                  |                               |
| 9 + Ca petroleum sulfonate                                                                                                                | 0.1                                                  | 36.8                          |
| 10 P <sub>2</sub> S <sub>5</sub> treated reaction product of ammonium hydrosulfide-hydrogen sulfide with topped, crude isophorone bottoms | 0.1                                                  |                               |
| 11 + Ca salt of alkyl phenolformaldehyde condensation product                                                                             | 0.2                                                  |                               |
| 12 + Ca petroleum sulfonate                                                                                                               | 0.1                                                  | 37.4                          |

<sup>1</sup> All oxidation products corrected to 1500 ml. oxygen absorbed per 100 g. of oil, assuming amount of product is proportioned to oxygen adsorbed.

The doped and undoped oils were further tested by a test known as the Thrust Bearing Corrosion test (described in the National Petroleum News, September 17, 1941, pp. R-294-296) which is carried out as follows: A hardened steel disc is made to rotate for 20 hours under constant pressure against three flat copper-lead bearings. The bearings assembly rests in a steel cup filled with the oil to be tested and the temperature of the oil is maintained at a predetermined figure by thermostatic control. The bearings are weighed before and after the test, the difference in weight representing the loss sustained during the test.

TABLE II  
*Tests in thrust bearing corrosion machine*

[Fixed conditions Cu-Pb bearings, 20 hours duration, 125 p. s. i. Thrust, 2,400 R. P. M. A refined, undoped, commercial lubricating oil 64-67 S. U. at 210° F. was employed]

|   | Additive                                                                                                                               | Amount, per cent weight | 150° C. | 160° C. | Estimated approximated Critical Corrosion Temperature |
|---|----------------------------------------------------------------------------------------------------------------------------------------|-------------------------|---------|---------|-------------------------------------------------------|
| 1 | None                                                                                                                                   | -----                   | 74.6    | -----   | 115° C.                                               |
| 2 | Ca salt of alkyl phenol-formaldehyde Condensation                                                                                      | .2                      | 0.2     | 24.8    | 155-160° C                                            |
|   | +Ca petroleum sulfonate                                                                                                                | .1                      |         |         |                                                       |
| 3 | Ca salt of alkyl phenol-formaldehyde Condensation                                                                                      | .2                      |         |         |                                                       |
|   | +Ca petroleum sulfonate                                                                                                                | .1                      |         |         |                                                       |
|   | +P <sub>2</sub> S <sub>5</sub> treated reaction product of ammonium hydrosulfide-hydrogen sulfide with topped crude isophorone bottoms | .1                      | 1.2     | 1.6     | 150° C.                                               |

In addition to the above properties the addition of reaction products of this invention to mineral lubricating oils inhibits lacquer formation in engines operating under the most adverse conditions. Also reaction products of this invention can be used as valuable constituents of heavy duty oils, motor oils, Diesel oils, aviation oils, turbine oil, synthetic oils and the like because of their anti-corrosion, antioxidation, and antiwear properties. Besides their utility as lubricating oil additives, reaction products of this invention are useful as anti-oxidants for natural and synthetic rubber and other organic materials which are subject to oxidation deterioration. The amount of additive used can be varied over wide limits but generally it is not necessary to use more than 5% by weight of the reaction product and preferably only between about 0.1 to 2.0% by weight is added to base lubricants.

Because of its synergistic effect the reaction product of this invention can be combined with other additives in lubricants, such as, blooming agents, pour point depressants or viscosity improvers, extreme pressure agents, antifoaming agents and the like. Among the specific additives which can be used are oil-soluble detergents which include oil-soluble salts of various bases with detergent forming acids. Such bases include metal as well as organic bases. Metallic bases include those of the alkali metals, Cu, Mg, Ca, Sr, Ba, Zn, Cd, Al, Sn, Pb, Cr, Mn, Fe, Ni, Co, etc. Organic bases include various nitrogen bases as primary, secondary, tertiary and quaternary amines.

Examples of detergent forming acids are the various fatty acids of, say, 10 to 30 carbon atoms,

wool fat acids, paraffin wax acids (produced by oxidation of paraffin wax) chlorinated fatty acids, rosen acids, aromatic carboxylic acids including aromatic fatty acids, aromatic hydroxy fatty acids, paraffin wax benzoic acids, various alkyl salicylic acids, phthalic acid monoesters, aromatic keto acids, aromatic ether acids, diphenols as di-(alkyl-phenol) sulfides and disulfides, methylene bis alkylphenols; sulfonic acids such as may be produced by treatment of alkyl aryl hydrocarbons or high boiling petroleum oils with sulfuric acid; sulfuric acid mono-esters; phosphoric, arsonic and antimony acid mono and diesters, including the corresponding thio phosphoric, arsonic and antimony acids; phosphonic and arsonic acids and the like.

Additional detergents are the alkaline earth phosphate diesters, including the thiophosphate diester; the alkaline earth diphenolates, specifically the calcium and barium salts of diphenol mono and poly sulfides.

Non-metallic detergents include compounds such as the phosphatides such as lecithin and cephalin, certain fatty oils as rapeseed oils, volto-lized fatty or mineral oils and the like.

An excellent metallic detergent for the present purpose is the calcium salt of oil-soluble petroleum sulfonic acids. This may be present advantageously in the amount of about 0.025% to 0.2% sulfate ash. Also alkaline metal salts of alkyl phenol-aldehyde condensation reaction products are excellent detergents.

Antioxidants comprise several types, for example, alkyl phenols such as 2,4,6 trimethyl phenol, penta methyl-phenol, 2,4 dimethyl-6-tertiary-butyl phenol, 2,4 - dimethyl - 6 - octyl phenol, 2,6 - di-tertiary-butyl-4-methyl-phenol, 2,4,6 tritertiary-butyl phenol and the like; amino phenols as benzyl amino phenols; amines such as dibutyl-phenylene diamine, diphenyl amine, phenyl - beta - naphthylamine, phenyl - alpha - naphthylamine, dinaphthyl amine.

Corrosion inhibitors or anti-rusting compounds may also be present such as dicarboxylic acids of 16 and more carbon atoms; alkali metal and alkaline earth salts of sulfonic acids and fatty acids; organic compounds containing an acidic radical in close proximity to a nitrile, nitro or nitroso group (e. g. alpha cyano stearic acid).

Extreme pressure agents which may be used comprise: esters or phosphorus acids such as tri-aryl, alkyl hydroxy aryl, or aralkyl phosphates, thiophosphates or phosphites and the like; neutral aromatic sulfur compounds of relatively high boiling temperatures such as diaryl sulfides, diaryl disulfides, alkyl aryl disulfides, e. g. diphenyl sulfide, diphenol sulfide, dicresol sulfide, dixylenol sulfide, methyl butyl diphenol sulfide, dibenzyl sulfide, corresponding di- and tri-sulfides, and the like; sulfurized fatty oils or esters of fatty acids and monohydric alcohols, e. g. sperm oil, jojoba oil, etc.; in which the sulfur is strongly bonded; sulfurized long chain olefins such as may be obtained by dehydrogenation or cracking of wax; sulfurized phosphorized fatty oils or acids, phosphorus acid esters having sulfurized organic radicals, such as esters of phosphoric or phosphorus acids with sulfurized hydroxy fatty acids; chlorinated hydrocarbons, such as chlorinated paraffin, aromatic hydrocarbons, terpenes, mineral lubricating oil, etc.; or chlorinated esters of fatty acids containing the chlorine in position other than alpha position.

Additional ingredients may comprise oil-soluble 75 urea or thiourea derivatives, e. g. urethanes,

allophanates, carbazides, carbazones, etc.; polyisobutylene polymers, unsaturated polymerized esters of fatty acids and monohydric alcohols and other high molecular weight oil-soluble compounds.

Depending upon the additive used and conditions under which it is used, the amount of additive used may vary from 0.01 to 2% or higher. However, substantial improvement is obtained by using amounts ranging from 0.1 to 0.5% in combination with phosphorous sulfide-unsaturated cyclic ketone reaction products of this invention.

The novel reaction products of this invention, in addition to being excellent lubricating oil improving agents, are potent oxidation inhibitors for fuels, natural and synthetic rubber, wax coating compositions and other organic materials.

It is to be understood that while the features of the invention have been described and illustrated in connection with certain specific examples, the invention, however, is not to be limited thereto or otherwise restricted, except by the prior art and the scope of the appended claims.

I claim as my invention:

1. A lubricant comprising a major amount of a mineral lubricating oil and a minor amount, sufficient to stabilize said oil against oxidation and corrosion deterioration, of a reaction product obtained by first reacting an organic compound with hydrogen sulfide and ammonium hydrosulfide at room temperature and treating the resulting reaction product with an inorganic compound selected from the group consisting of phosphorus sulfide, sulfur halide, elemental sulfur and alkali polysulfide at a temperature of at least 150° C.

2. A lubricant comprising a major amount of mineral lubricating oil and a minor amount, sufficient to stabilize said oil against oxidation and corrosion deterioration, of a reaction product obtained by first reacting an organic compound with hydrogen sulfide and ammonium hydrosulfide, at between about room temperature to about 100° C. and treating the resulting reaction product with an inorganic compound selected from the group consisting of phosphorus sulfide, sulfur halide, elemental sulfur and alkali polysulfide at a temperature of between about 150° to about 170° C.

3. A lubricant comprising a major amount of mineral lubricating oil and a minor amount, sufficient to stabilize said oil against oxidation and corrosion deterioration, of a reaction product obtained by first reacting an oxygen-containing organic compound with hydrogen sulfide and ammonium hydrosulfide, at between about room temperature to about 100° C. and treating the resulting reaction product with an inorganic compound selected from the group consisting of phosphorus sulfide, sulfur halide, elemental sulfur and alkali polysulfide at a temperature of between about 150° to about 170° C.

4. A lubricant comprising a major amount of mineral lubricating oil and a minor amount, sufficient to stabilize said oil against oxidation and corrosion deterioration, of a reaction product obtained by first reacting a high molecular weight hydrocarbon with hydrogen sulfide and ammonium hydrosulfide, at between about room temperature to about 100° C. and treating the resulting reaction product with an inorganic compound selected from the group consisting of phosphorus sulfide, sulfur halide, elemental sulfur and alkali polysulfide at a temperature of between about 150° to about 170° C.

5. A lubricant comprising a major amount of mineral lubricating oil and a minor amount, sufficient to stabilize said oil against oxidation and corrosion deterioration, of a reaction product obtained by first reacting a saturated cyclic ketone having at least 12 carbon atoms with hydrogen sulfide and ammonium hydrosulfide, at between about room temperature to about 100° C. and treating the resulting reaction product with an

10 inorganic compound selected from the group consisting of phosphorus sulfide, sulfur halide, elemental sulfur and alkali polysulfide at a temperature of between about 150° to about 170° C.

6. A lubricant comprising a major amount of mineral lubricating oil and a minor amount, sufficient to stabilize said oil against oxidation and corrosion deterioration, of a reaction product obtained by first reacting an unsaturated cyclic ketone having at least 12 carbon atoms with hydro-

15 gen sulfide and ammonium hydrosulfide, at between about room temperature to about 100° C. and treating the resulting reaction product with an inorganic compound selected from the group consisting of phosphorus sulfide, sulfur halide, elemental sulfur and alkali polysulfide at a tem-

20 perature of between about 150° to about 170° C.

7. A lubricant comprising a major amount of mineral lubricating oil and a minor amount, sufficient to stabilize said oil against oxidation and corrosion deterioration, of a reaction product obtained by first reacting a wax olefin with hydro-

25 gen sulfide and ammonium hydrosulfide, at between about room temperature to about 100° C. and treating the resulting reaction product with an inorganic compound selected from the group consisting of phosphorus sulfide, sulfur halide, elemental sulfur and alkali polysulfide at a tem-

30 perature of between about 150° to about 170° C.

8. A lubricant comprising a major amount of mineral lubricating oil and a minor amount, of

35 from 0.1% to 5% by weight, of a reaction product obtained by first reacting a saturated cyclic ketone having at least 12 carbon atoms with hydro-

40 gen sulfide and ammonium hydrosulfide at be-

45 tween about room temperature and 100° C. and treating the resulting reaction product with phosphorus pentasulfide at a temperature of at

50 least 150° C.

9. A lubricant comprising a major amount of mineral lubricating oil and a minor amount, of

55 from 0.1% to 5% by weight, of a reaction product obtained by first reacting an unsaturated cyclic

60 ketone having at least 12 carbon atoms with hydro-

65 gen sulfide and ammonium hydrosulfide at be-

70 tween about room temperature and 100° C. and treating the resulting reaction product with phosphorus pentasulfide at a temperature of at

75 least 150° C.

10. A lubricant comprising a major amount of mineral lubricating oil and a minor amount, of

70 from 0.1% to 5% by weight, of a reaction product obtained by first reacting a wax olefin with hydro-

75 gen sulfide and ammonium hydrosulfide at be-

75 tween about room temperature and 100° C. and treating the resulting reaction product with ele-

## 15

mental sulfur at a temperature of at least 150° C.

12. A lubricant comprising a major amount of mineral lubricating oil and a minor amount, of from 0.1% to 5% by weight, of a reaction product obtained by first reacting an unsaturated cyclic ketone having at least 12 carbon atoms with hydrogen sulfide and ammonium hydrosulfide at between about room temperature and 100° C. and treating the resulting reaction product with elemental sulfur at a temperature of at least 150° C.

13. A lubricant comprising a major amount of mineral lubricating oil and a minor amount, of from 0.1% to 5% by weight, of a reaction product obtained by first reacting a wax olefin with hydrogen sulfide and ammonium hydrosulfide at between about room temperature and 100° C. and treating the resulting reaction product with elemental sulfur at a temperature of at least 150° C.

14. A compounded lubricant comprising a major amount of mineral lubricating oil and containing an active amount of calcium salt of alkyl phenol formaldehyde condensation reaction product, calcium salt of petroleum sulfonic acid as detergents, and a small amount of from 0.1% to 5% by weight of a reaction product obtained by first reacting an organic compound with hydrogen sulfide and ammonium hydrosulfide, at between about room temperature to about 100° C. and treating the resulting reaction product with an inorganic compound selected from the group consisting of phosphorus sulfide, sulfur, halide, elemental sulfur and alkali polysulfide at a temperature of between about 150° to about 170° C.

15. Process of producing a stable, non-corrosive oil-soluble liquid hydrocarbon lubricant additive which comprises reacting in a solvent an organic compound with hydrogen sulfide and ammonium hydrosulfide at between about room temperature to about 100° C., and treating the resulting reaction product with phosphorus pentasulfide at between about 150° to 170° C. removing the solvent and adding from 0.1% to 5% of said final reaction product to a lubricant.

16. Process of producing a stable, non-corrosive oil-soluble liquid hydrocarbon lubricant additive which comprises reacting in a solvent an organic compound with hydrogen sulfide and ammonium hydrosulfide at between about room temperature to about 100° C., and treating the resulting reaction product with elemental sulfur at between about 150° to 170° C. removing the solvent and adding from 0.1% to 5% of said final reaction product to a lubricant.

17. A lubricant comprising a major amount of mineral lubricating oil and a minor amount, sufficient to stabilize said oil against deterioration, of a salt of a reaction product obtained by first reacting an unsaturated cyclic ketone having at least 12 carbon atoms with hydrogen sulfide in the presence of ammonium hydrosulfide, at between about room temperature and about

## 16

100° C. and treating the resulting reaction product with an inorganic compound selected from the group consisting of phosphorus sulfide, sulfur halide, elemental sulfur and alkali polysulfide at a temperature of between about 130° and about 170° C., and thereafter neutralizing said reaction product to form the salt.

18. A lubricant comprising a major amount of mineral lubricating oil and a minor amount, sufficient to stabilize said oil against deterioration, of a salt of a reaction product obtained by first reacting a saturated cyclic ketone having at least 12 carbon atoms with hydrogen sulfide-ammonium hydrosulfide, at between about room temperature and about 100° C. and treating the resulting reaction product with an inorganic compound selected from the group consisting of phosphorus sulfide, sulfur halide, elemental sulfur and alkali polysulfide at a temperature of between about 150° and about 170° C., and thereafter neutralizing said reaction product to form the salt.

19. A lubricant comprising a major amount of mineral lubricating oil and a minor amount, sufficient to stabilize said oil against deterioration, of a salt of a reaction product obtained by first reacting an oxygen-containing organic compound with hydrogen sulfide-ammonium hydrosulfide, at between about room temperature and about 100° C. and treating the resulting reaction product with an inorganic compound selected from the group consisting of phosphorus sulfide, sulfur halide, elemental sulfur and alkali polysulfide at a temperature of between about 150° and about 170° C., and thereafter neutralizing said reaction product to form the salt.

20. A composition consisting of the reaction product obtained by first reacting an unsaturated cyclic ketone having at least 12 carbon atoms with hydrogen sulfide-ammonium hydrosulfide at between about room temperature and about 100° C., treating the resulting reaction product with phosphorus pentasulfide at a temperature of between about 150° and about 170° C. and neutralizing said reaction product with an alkaline earth metal.

DAVID E. ADELSON.

## REFERENCES CITED

The following references are of record in the file of this patent:

## UNITED STATES PATENTS

| Number    | Name                   | Date          |
|-----------|------------------------|---------------|
| 2,266,325 | Lazar et al. -----     | Dec. 16, 1941 |
| 2,353,491 | Oberright -----        | July 11, 1944 |
| 2,361,805 | Wilson -----           | Oct. 31, 1944 |
| 2,383,497 | Ott et al. -----       | Aug. 28, 1945 |
| 2,413,648 | Otto -----             | Dec. 31, 1946 |
| 2,419,153 | Musselman et al. ----- | Apr. 15, 1947 |

**Certificate of Correction**

**Patent No. 2,489,249**

**November 29, 1949**

**DAVID E. ADELSON**

It is hereby certified that error appears in the printed specification of the above numbered patent requiring correction as follows:

Column 16, line 5, for "130°" read 150°;  
and that the said Letters Patent should be read with this correction therein that the same may conform to the record of the case in the Patent Office.

Signed and sealed this 9th day of May, A. D. 1950.

**[SML]**

**THOMAS F. MURPHY,**  
*Assistant Commissioner of Patents.*